

April 12, 1927.

1,624,762

A. RÜTTENAUER ET AL

REFLECTOR LAMP

Filed May 14, 1926

Fig. 1.



Fig. 2.



Inventors:  
Alfred Rüttenauer,  
Georg Gaidies,  
by *Alfred S. Lunt*,  
Their Attorney.

## UNITED STATES PATENT OFFICE.

ALFRED RÜTTENAUER, OF CHARLOTTENBURG, BERLIN, AND GEORG GAIDIES, OF PANKOW, BERLIN, GERMANY, ASSIGNORS TO GENERAL ELECTRIC COMPANY, A CORPORATION OF NEW YORK.

## REFLECTOR LAMP.

Application filed May 14, 1926, Serial No. 109,160, and in Germany June 26, 1925.

In electric incandescent lamps attempts have been made to utilize a portion of the bulb of the lamp as a reflector by applying to it a thin silver coating to make the lamp 5 a searchlight. This simple and advantageous method for securing a directed beam of light can not be used in lamps in which the bulbs, on account of their small size or the use of a high wattage filament, heat up to 10 more than 250 degrees C. for example, because the means which have been proposed to protect the silver coating against oxidation do not withstand such high heating of the bulb for any length of time. For example, aluminum bronze, frequently used 15 as a protective coating for the silver, will withstand temperatures of the bulb of only about 150 degrees C. for at even lower temperature the aluminum bronze layer swells 20 and finally scales off. The many lacings proposed for the protection of the silver coating are as a whole not essentially more heat resistant than any aluminum bronze layer. The aquadag layer sometimes used in reflector automobile lamps and made from a 25 colloidal carbon solution does stand somewhat higher temperatures, but at temperatures of about 250 degrees C. is on the point of vaporizing, so that in automobile lamps 30 of high candle power a coating of the interior of the automobile headlight by vaporization of the protective layer cannot be avoided. Even when the silver coating is covered on the outside with nickel with the 35 interposition of a copper coating the bulb temperature must not exceed approximately 200 degrees C. or at most 250 degrees C. as otherwise damage or flaking off of the outer nickel protective layer takes place. Such 40 a protective layer also has the further disadvantage that if a very fine hole or fissure in the outer nickel layer is present or develops, yellow spots are produced on the silver mirror by the oxidation of the copper. 45 It has also been proposed to protect the silver coating by a ceramic coating consisting of a mass of very hard silicate. This coating, though it is highly refractory, has the disadvantage that it is porous and allows 50 especially at high temperatures, the oxygen of the air to seep through to the silver coating, causing discoloration or spotting of the silver coating. A further disadvantage of this hard ceramic protective coating is that it can be made only in a comparatively thick 55 and irregular layer, which naturally makes the lamp unnecessarily heavy and detracts from its appearance.

This invention provides a means of so protecting a silver coating on the bulb of an 60 electric lamp that the bulb can, in operation, be raised, without danger to the coating, to far higher temperatures, even above 400 degrees C. To this end, the thin silver layer employed for the reflector is protected by an 65 enamel layer fused over it. The enamel layer, by the fusion of its particles produced during the application of the layer, attains a smooth surface which hermetically seals off the silver coating from the outside, so 70 that even with a higher heating of the bulb than has heretofore been feasible, the entrance of air to the silver coating becomes impossible. The smooth surface of this protective layer and the fact that it can 75 easily be made of very slight thickness has as the further advantage that the lamp is not impaired in its appearance and has only a slightly greater weight than an ordinary 80 silver coated lamp.

In the accompanying drawing we have illustrated as one example of a lamp embodying our invention, an automobile lamp of which Fig. 1 is an elevation and Fig. 2 a section through a part of the coated part of 85 the bulb. In this particular lamp the glass bulb 1 has on a portion of its surface a reflecting layer or coating 2 of some metal, such as silver, covered with a smooth protective layer 3 of enamel fused in place over 90 the silver reflector to hermetically seal the silver coating from the air. As a result, the reflector is protected from the action of the air even though the bulb attains a temperature as high as 400 degrees C. 95

In the manufacture of a lamp in accordance with our invention, the following process can be followed:

The lamp bulb 1 or even a completely finished lamp is first carefully cleaned and 100 then dipped for some minutes into one or several silver plating baths to apply the silver coating and then allowed to dry. Then the bulb or lamp is put into a bath of an enamel in suspension and preferably containing some clouding means dissolved in alcohol, or else the suspension is applied to the bulb by squirting, pouring or painting.

It is also possible to apply the enamel by dusting on a dry, easily fusible enamel powder. The applied enamel layer is finally heated in a furnace or by gas burners for some minutes to the burning in temperature of the enamel, whereupon the separate particles of the enamel are fused and form a smooth, uniform surface even when the enamel is in a very thin layer. In order to avoid deformation of the lamp bulb when the enamel is burned in, there must naturally be chosen an enamel which is suitable for the bulb glass. If the lamp bulb consists, for example, of hard glass such as a difficultly fusible magnesia or boro silicate glass, then most of the enamels on the market can be directly applied. If, however, the lamp bulb consists of the ordinary lead glass with a melting point of 500 to 550 degrees C., then it is preferable to use an enamel having a burning in temperature which does not exceed 480 degrees C.

The lamps provided with the new enamel protective layer can permanently stand temperatures of more than 400 degrees C. without damage or changes in the consistency of the protective layer or of the underlying silver coating. As a result, the invention can advantageously be employed wherever a good concentration is desired of the light of a lamp which in operation reaches a high heat, such as projection lamps, automobile lamps, and searchlight lamps. It is immaterial whether the lamp is a vacuum incandes-

cent lamp, a gas filled incandescent lamp, or an arc lamp having a bulb.

While we have described as one embodiment of our invention a lamp having a bulb of which a portion is made into a reflector by a coating of silver, our invention is not restricted to such embodiment, but is applicable to searchlight and similar reflectors and to other devices in which a sheet or body of glass coated with silver is subjected to temperatures high enough to cause spotting or tarnishing of an unprotected silver coating.

What we claim as new and desire to secure by Letters Patent of the United States is:

1. An electric lamp comprising a bulb, and a silver coating on the bulb protected by a fused enamel layer covering and hermetically sealing the coating.

2. A reflector comprising a sheet of glass and a coating of highly reflecting metal susceptible to oxidation at high temperature adherent to the glass and hermetically sealed from the air by a protective layer of fused enamel.

3. A reflector comprising a curved sheet of glass and a coating of silver on its surface protected by an air tight smooth layer of enamel fused in place on the glass and over said coating.

In witness whereof, we have hereunto set our hands this 27th day of April, 1926.

ALFRED RÜTTENAUER.  
GEORG GAIDIES.